



US005407722A

**United States Patent** [19]

Peake, III et al.

[11] **Patent Number:** 5,407,722[45] **Date of Patent:** \* Apr. 18, 1995

[54] **LOOP-TYPE TEXTILE FASTENER FABRIC, METHOD OF PRODUCING SAME AND PROCESS OF TREATING SAME**

[75] Inventors: William L. Peake, III; Robert T. Spillane; Phillip D. McCartney; Paul R. Huebner, all of Greensboro, N.C.

[73] Assignee: Guilford Mills, Inc., Greensboro, N.C.

[\*] Notice: The portion of the term of this patent subsequent to Dec. 7, 2010 has been disclaimed.

[21] Appl. No.: 138,335

[22] Filed: Oct. 18, 1993

**Related U.S. Application Data**

[63] Continuation-in-part of Ser. No. 34,088, Mar. 22, 1993, Pat. No. 5,267,453, which is a continuation-in-part of Ser. No. 711,201, Jun. 6, 1991, Pat. No. 5,214,942.

[51] Int. Cl.<sup>6</sup> ..... D04B 23/08; A44B 18/00; B32B 3/06; B32B 7/00

[52] U.S. Cl. ..... 428/88; 428/92; 428/95; 428/100; 428/230; 428/253; 428/257; 428/258; 428/259; 66/194; 66/193

[58] **Field of Search** ..... 428/88, 95, 92, 100, 428/230, 253, 257, 258, 259; 66/193, 194

**References Cited****U.S. PATENT DOCUMENTS**

|           |         |                       |       |          |
|-----------|---------|-----------------------|-------|----------|
| 3,594,873 | 7/1971  | Hockmeyer, Jr. et al. | ..... | 66/194 X |
| 3,597,941 | 8/1971  | Domazlice             | ..... | 66/194 X |
| 3,748,701 | 7/1973  | De Mestral            | ..... | 66/194 X |
| 3,943,981 | 3/1976  | De Brabander          | ..... | 66/194 X |
| 4,114,346 | 9/1978  | Kelly                 | ..... | 66/194 X |
| 4,338,800 | 7/1982  | Matsuda               | ..... | 66/194 X |
| 4,467,625 | 8/1984  | Kurz                  | ..... | 66/194 X |
| 4,557,774 | 12/1985 | Hoopengardner         | ..... | 66/194 X |
| 4,624,116 | 11/1986 | Rogers                | ..... | 66/194 X |
| 4,677,011 | 6/1987  | Matsuda               | ..... | 66/194 X |

|           |         |                 |       |          |
|-----------|---------|-----------------|-------|----------|
| 4,709,562 | 12/1987 | Matsuda         | ..... | 66/194 X |
| 4,714,096 | 12/1987 | Guay            | ..... | 66/194 X |
| 4,822,658 | 4/1989  | Pacione         | ..... | 66/194 X |
| 4,838,044 | 6/1989  | Matsuda et al.  | ..... | 66/194 X |
| 4,858,447 | 8/1989  | Matsuda         | ..... | 66/194 X |
| 4,881,383 | 11/1989 | Spillane et al. | ..... | 66/194 X |

**FOREIGN PATENT DOCUMENTS**

1204886 9/1967 United Kingdom

**OTHER PUBLICATIONS**

Guilford Mills, Inc. Warp Knitted Fabric Style No. 30000.

*Primary Examiner*—Patrick J. Ryan

*Assistant Examiner*—Richard P. Weisberger

*Attorney, Agent, or Firm*—Shefte, Pinckney & Sawyer

[57]

**ABSTRACT**

A lightweight warp knitted textile fabric suitable for use as the loop component of a hook-and-loop fastener is formed of a set of ground yarns knitted in a relatively stretchable construction with a set of loop-forming yarns formed in a stitch pattern producing elongated underlap loops extending outwardly from the technical back of the fabric which can be readily interengaged with the hook elements of a mating hook component without any necessity for brushing, napping or mechanically raising the loops. In one embodiment, a second set of loop-forming yarns is formed in a stitch pattern producing elongated loops extending outwardly from the technical face of the fabric which can be adhered to a backing material such as a carpet backing. In another embodiment, filling yarn is inserted weftwise in every fabric course. The fabric is preferably finished with a starch application to improve handleability during subsequent processing and, in the case of the second embodiment, a fluorocarbon composition is applied when the fabric will be adhered to a foam carpet backing to restrict foam penetration into the fabric interstices.

12 Claims, 3 Drawing Sheets



Fig. 1





Fig. 2

Fig.3



**LOOP-TYPE TEXTILE FASTENER FABRIC,  
METHOD OF PRODUCING SAME AND PROCESS  
OF TREATING SAME**

**CROSS-REFERENCE TO RELATED  
APPLICATION**

This is a continuation-in-part of U.S. patent application Ser. No. 08/034,088, filed Mar. 22, 1993, now U.S. Pat. No. 5,267,453 entitled **LOOP-TYPE TEXTILE FASTENER FABRIC AND METHOD OF PRODUCING SAME**, which is a continuation-in-part of U.S. patent application Ser. No. 07/711,201, filed Jun. 6, 1991, now U.S. Pat. No. 5,214,942 entitled **LOOP-TYPE TEXTILE FASTENER FABRIC AND METHOD OF PRODUCING SAME**.

**BACKGROUND OF THE INVENTION**

The present invention relates generally to fabric fasteners of the type commonly referred to as hook-and-loop fasteners. More particularly, the present invention relates to a novel warp-knitted loop-type textile fastener fabric and a method of producing such a fastener fabric on a warp knitting machine. A method of preparatory treatment of the fabric is also disclosed.

So-called hook-and-loop fasteners have gained considerable popularity over recent years. Such fasteners basically include two generally flat components attachable and detachable to and from face abutting relation with one another. Typically, each fastener component is of a textile fabric construction, the hook or "male" component having a fabric ground layer with a plurality of relatively stiff hook-shaped elements extending in upstanding relation from one face of the ground layer and the loop or "female" component similarly having a fabric ground layer with a plurality of relatively flexible pile-type loops extending outwardly from one face of the ground layer. In use, the hook and loop faces of the fastener components grippingly engage one another when pressed together in face abutting relation by penetration of the hook-shaped elements of the hook component into the loops at the opposing face of the loop component. The engagement between the hook and loop faces of the two components resists separation thereof until a threshold force is exerted on one component in a peeling-like fashion.

Typically, both components of conventional hook-and-loop fasteners have been of relatively heavyweight constructions. For example, many hook components utilize hook elements formed of relatively heavy denier inflexible synthetic monofilament yarns firmly secured in a similarly stiff inflexible ground fabric, to withstand repeated attachment and detachment to and from a mating loop component without excessive breakage of the hook elements or tearing of the ground fabric. Similarly, loop components commonly have a relatively stiff inflexible ground layer supporting elongated loops of multifilament synthetic yarns, which normally are brushed or napped to produce a plush-like loop surface wherein the individual filaments are mainly separated from one another, in order to maximize the available loops for engagement with the mating hook-like elements of the other fastener component. Thus, although a number of the individual filaments in the loops may be broken each time the hook and loop components are attached and then detached, the large number of available loops owing to the use of napped or brushed multifilament yarns enables the loop component to be repeat-

edly attached and detached to and from its mating hook component so that the fastener generally has a reasonably extended useful life.

Virtually without exception, conventional hook-and-loop fasteners are fabricated with each fastener component in the form of a relatively narrow width tape of indeterminate length. As such, hook-and-loop fasteners are susceptible to a wide variety of end uses, most often as a fastener or closure in various apparel items wherein the capability of the fastener components for repetitive attachment and detachment to and from one another is a virtual necessity.

However, a variety of other uses for hook-and-loop fasteners has also been proposed. For example, U.S. Pat. No. 4,822,658 discloses a carpet construction with a backing layer having plural downwardly projecting loops serving the dual purpose of providing resiliency to the underside of the carpet in the nature of underpadding while also being adapted for engagement with a hook-type fastener tape affixed to a floor surface for purposes of securing the carpeting in place on the floor. To economically produce this product, a loop-type fastener component for use as the backing layer must be fabricated in the same widths as carpeting is typically fabricated, e.g., twelve-foot widths or greater. However, no conventional hook-and-loop fastener constructions are known to be fabricated in such widths to be suitable for the use contemplated by this patent. Moreover, since the looped underlayer of this carpet construction would not be repeatedly engaged with and disengaged from the mating hook fastener tape but instead would generally perform a one-time use, the loop components of conventional hook-and-loop fasteners of the type described above would not be optimally suitable for use in such carpet construction in any event.

Other uses which have been proposed for hook-and-loop fasteners include the formation of closures in disposable or one-time use products, such as diapers and incontinence garments, for which the above-described conventional hook-and-loop fasteners would also be generally inappropriate.

**SUMMARY OF THE INVENTION**

It is accordingly an object of the present invention to provide a novel loop component for use in a hook-and-loop fastener which is suitable for uses wherein repeated attachment and detachment to and from a mating hook component is generally unnecessary. A particular object of the present invention is to provide such a loop component which is specifically suitable for use as a backing in a carpet construction such as disclosed in the aforementioned U.S. Pat. No. 4,822,658, closures for disposable articles, and in other one-time and light-duty uses.

It is a further object of the present invention to provide a loop component for a hook-and-loop fastener of a warp knitted textile fabric construction wherein the loop-forming yarn is knitted in a stitch pattern causing the surface loops to be elongated and to extend outwardly from the fabric without brushing, napping or otherwise mechanically raising the loops. A more specific object is to provide such a loop component utilizing a relatively fine denier synthetic yarn for formation of the surface loops on one face of the fastener component.

An additional object of the present invention is to provide a novel warp knitting method for fabricating

the loop fastener component of the present invention. Another object is to provide a process for preparatory treatment of the fabric to improve its handleability and performance during subsequent processing operations.

Briefly summarized, the present invention provides a textile fabric having one face adapted to be adhered to a backing material (e.g., the backing surface of a carpet) and a set of pile-like loops at the other face adapted for mated engagement with hooking elements of another fabric for use in a two-component fabric fastener of the hook-and-loop type. Basically, the fabric fastener component of the present invention includes a ground layer formed of a ground yarn and a loop-forming yarn forming the set of loops and extending outwardly from the aforesaid other face of the ground layer. According to one aspect of the present invention, the fastener fabric is formed of a warp knitted construction with the pile-like loops appearing at either the technical face of the fabric or the technical back of the fabric or at both fabric sides. More specifically, the warp knitted fastener component includes yarns formed in needle loops arranged in longitudinally extending wales and transversely extending courses including a set of ground yarns formed in a stitch pattern of needle loops which is relatively stretchable in the warpwise extent of the fabric and a set of loop-forming yarns knitted with the ground yarns in needle loops in spaced courses and spaced wales wherein the ground yarn needle loops are formed and in pile-like loops extending outwardly from the aforesaid other face of the fabric between the needle loops of the loop-forming yarns.

Preferably, each loop-forming yarn is formed in needle loops aligned with one another in spaced courses of a common wale. For example, the loop-forming yarns may be warp knitted in a 1-0, 3-4, 6-7, 3-4 stitch pattern or in a 1-0, 3-4 stitch pattern. It is also preferred that the ground yarns are formed in a 2-3, 1-0 stitch pattern or in a 1-0, 2-3 stitch pattern.

A weft inserted filling yarn may be formed to extend coursewise in at least some of the fabric courses, preferably in substantially every course.

Optionally, a second set of loop-forming yarns may be knitted with the ground yarns of the fabric in needle loops in spaced courses and spaced wales wherein the ground yarn needle loops are formed and in pile-like loops extending outwardly from the first aforesaid one face of the fabric between the needle loops of the second loop-forming yarns.

The present invention also contemplates a method of producing a warp knitted textile fabric suitable for use as the loop component of a hook-and-loop type fastener. Basically, the present method includes the steps of warp knitting a set of ground yarns on one guide bar of a warp knitting machine having at least two guide bars to form a ground layer of the fabric in a relatively stretchable construction while simultaneously warp knitting a set of loop-forming yarns on the other guide bar of the knitting machine to form raised pile-like loops at one surface of the fabric.

According to one aspect of the present method, the loop-forming yarns are knitted by alternately forming needle loops of the loop-forming yarns on selected needles of the knitting machine's needle bar and interveningly holding the loop-forming yarns in a non-knitting manner on, and then releasing the loop-forming yarns without stitch formation from, other needles spaced from the selected needles to form the respective out-

wardly-extending loops between the respective needle loops of the loop-forming yarns.

In the preferred embodiment of the present method, the ground yarns are warp knitted in a 2-3, 1-0 stitch pattern or in a 1-0, 2-3 stitch pattern and the loop-forming yarns are warp knitted in a 1-0, 3-4, 6-7, 3-4 stitch pattern or in a 1-0, 3-4 stitch pattern. A filling yarn may be inserted weftwise in at least some or, more preferably, substantially all of the courses of the fabric.

Another aspect of the present invention provides a process for treating the aforescribed stretchable loop-type textile fastener fabrics to prepare the fabrics for subsequent processing, including adhesion of the fabric to a foam backing layer, e.g., the foam backing of a carpet. Basically, the treating process comprises the steps of applying a stiffening agent to the fabric to temporarily improve its handleability, the stiffening agent being readily broken and releasable from the fabric during subsequent processing as a result of manipulation, bending and like handling of the fabric so that the lengthwise stretchability of the fabric is not permanently impaired. For example, the stiffening agent may be a starch. A foam resistant agent is also applied to the fabric for the purpose of partially resisting adhesion of the foam to the fabric thereby to restrict foam penetration into the fabric structure so that the fabric retains a desirable degree of its lengthwise stretchability after adhesion to the foam backing layer. For example, the foam resistant agent may be a fluorocarbon composition, preferably having both water resistant and oil resistant properties, e.g., a mixture of a water-resistant fluorocarbon and an oil resistant fluorocarbon. Preferred fluorocarbons for this purpose are the FC 247 fluorocarbon manufactured and sold by 3-M Company (Minnesota Mining and Manufacturing Company) of St. Paul, Minn., and the ZONAL 8070 fluorocarbon manufactured and sold by CIBA Company of Greensboro, N.C.

The stiffening agent is contained in a bath wherein the content of the stiffening agent is in the range of approximately 10 percent to 40 percent of the weight of the bath. The stiffening agent is applied to the fabric either by spraying the bath onto the face of the fabric to be subsequently adhered to the foam backing layer, in which case a higher percentage stiffening agent content is preferred, or by passing the fabric through the bath, e.g., in a padding process, in which case the bath may have a stiffening agent content at the lower end of the aforementioned range. The fluorocarbon composition, or other foam resistant agent, is also prepared in the form of a bath preferably having a content of the foam resistant agent in the range of approximately 0.25 percent to 8 percent of the weight of the bath.

#### BRIEF DESCRIPTION OF THE DRAWINGS

FIG. 1 is a diagram showing individually the stitch pattern for the ground and loop-forming yarns carried out by a warp knitting machine in knitting one preferred embodiment of the present fabric according to the method of the present invention;

FIG. 2 is a composite diagram thereof; and

FIG. 3 is a diagram similar to FIG. 1 showing individually the stitch pattern for the ground and loop-forming yarns carried out by a warp knitting machine, including the weft insertion of a filling yarn, in knitting another preferred embodiment of the present fabric according to the method of the present invention.

## DESCRIPTION OF THE PREFERRED EMBODIMENT

As explained more fully herein, the preferred embodiments of the fabric of the present invention are produced, and the method of the present invention is carried out, on a warp knitting machine which may be of any conventional type of an at least two-bar construction having two or more yarn guide bars and a needle bar, e.g., a conventional tricot warp knitting machine. The construction and operation of such machines are well known in the warp knitting art and need not herein be specifically described and illustrated. In the following description of exemplary embodiments of the invention, the yarn guide bars of a two-bar knitting machine are identified as "top" and "bottom" guide bars and the yarn guide bars of a three-bar knitting machine are identified as "top," "middle" and "bottom" guide bars for references purposes only and not by way of limitation. As those persons skilled in the art will understand, such terms equally identify knitting machines whose guide bars may be referred to as "front," "middle" and "back" guide bars, which machines of course are not to be excluded from the scope and substance of the present invention. As further used herein, the "bar construction" of a warp knitting machine refers to the number of yarn guide bars of the machine, while the "bar construction" of a warp knitted fabric refers to the number of different sets of warp yarns included in the fabric, all as is conventional terminology in the art.

Referring now initially to FIGS. 1 and 2 of the accompanying drawings, one particular embodiment of the present textile fabric is illustrated as preferably warp knitted of a three-bar construction on a three-bar warp knitting machine according to the present method. As is conventional, the needle bar of the warp knitting machine carries a series of aligned knitting needles, while each guide bar of the machine carries a series of guide eyes, the needle and guide bars preferably having the same gauge, i.e., the same number of needles and guide eyes per inch. According to the illustrated embodiment of the present fabric, the top guide bar of the machine is threaded on alternating guide members with a first set of loop-forming yarns 14 delivered from a warp beam (not shown), the middle guide bar is threaded on alternating guide members with a set of ground yarns 12 delivered from another warp beam (also not shown), and the bottom guide bar is similarly threaded on alternating guide members with a second set of loop-forming yarns 10 supplied from a third warp beam (also not shown). For this purpose, each of the bottom, middle and top yarn guide bars has every alternate guide eye empty and every intervening guide eye threaded with a respective ground or loop-forming yarn 10, 12 or 14, commonly referred to as a "one out, one in" threading arrangement. As more fully explained hereinafter, the threading arrangement of the three guide bars is set up in conjunction with the stitch patterns of the three sets of yarn to deliver the ground and loop-forming yarns 10, 12, 14 to every alternate needle of the needle bar during the formation of alternate fabric courses and, then, to deliver the ground yarn 12 to every alternate needle of the needle bar while delivering the loop-forming yarns 10, 14 to every intervening needle during the formation of intervening fabric courses.

It is contemplated that a variety of yarns may be suitable for use as the ground and loop-forming yarns.

For example, any of a variety of conventional multifilament synthetic yarns, particularly polyester and nylon yarns, would be suitable for use as any or all of the ground and loop-forming yarns. Texturized yarns offer the additional advantage of enhancing the desired stretchability of the fabric. The denier of the yarns may vary depending upon the desired weight of the fabric per unit fabric dimension (ounces per square yard).

In the accompanying FIG. 1, the stitch constructions of the ground and loop-forming yarns 10, 12, 14, as carried out by the respective lateral traversing movements of the guide bars of the knitting machine according to one possible embodiment of the present fabric and method, are illustrated individually in a traditional dot or point diagram format, wherein the individual points 15 represent the needles of the needle bar of the knitting machine in the formation of several successive fabric courses C across several successive fabric wales W. According to this embodiment, the bottom (or back) guide bar of the warp knitting machine manipulates the second set of loop-forming yarns 10 as they are fed from their respective warp beam to traverse laterally back and forth relative to the needle bar of the machine alternately to stitch the loop-forming yarns 10 on alternate needles 15A and then to lay the yarns 10 without stitch formation about the intervening needles 15B in a repeating 1-0, 3-4 stitch pattern, as indicated at I of FIG. 1. Similarly, the top (or front) guide bar simultaneously manipulates the first set of loop-forming yarns 14 as they are fed from their respective warp beam to traverse relative to the needle bar alternately to stitch the loop-forming yarns 14 on the same alternating needles 15A and then to lay the yarns 14 without stitch formation about spaced intervening needles 15B in a repeating 1-0, 3-4, 6-7, 3-4 stitch pattern, as indicated at III of FIG. 1. Simultaneously, the middle guide bar of the knitting machine manipulates the set of ground yarns 12 as they are fed from their respective warp beam to traverse relative to the needle bar in opposition to the top and bottom guide bars to stitch the ground yarns 12 on the same alternating needles 15A in a repeating 2-3, 1-0 stitch pattern, as indicated at II in FIG. 1. The respective simultaneous stitch patterns of the ground and loop-forming yarns 10, 12, 14 are shown in a composite dot diagram in FIG. 2.

As will thus be understood, the ground and loop-forming yarns 10, 12, 14 are interknitted with one another by formation of respective needle loops 10n, 12n, 14n of the yarns in alternating wales W1 and alternating courses C1 of the resultant fabric, without any needle loops of any of the yarns being formed in the intervening wales W2 and only needle loops 12n of the ground yarns 12 being formed in the alternating wales W1 of the intervening courses C2. More specifically, the stitch construction of the first loop-forming yarns 10 forms needle loops 10n thereof only in alternating wales W1 of alternating courses C1, each individual loop-forming yarn 10 having its respective needle loops 10n formed in alternating courses C1 and in a single common wale W1 with connecting underlap extents 10u extending between the successive needle loops 10n generally in the intervening courses C2. The ground yarns 12 are formed only in the alternating wales W1, each individual ground yarn 12 having its respective needle loops 12n alternating every course C between adjacent alternate wales W1 across the one intervening wale W2 across which underlaps 12u of the ground yarn extend diagonally back and forth in a substantially coursewise

direction between the successive needle loops  $12n$ . The stitch construction of the loop-forming yarns  $14$  form them in needle loops  $14n$  appearing only in the alternating courses  $C1$  and in the alternating wales  $W1$ , each individual loop-forming yarn  $14$  having its respective needle loops  $14n$  formed in the alternating courses  $C1$  in a single common wale  $W1$  with connecting underlap extents  $14u$  extending between the successive needle loops  $14n$  generally in the intervening courses  $C2$ .

As those persons skilled in the art will recognize, the respective stitch patterns followed by the loop-forming yarns  $10,14$  cause each such yarn to be traversed during the formation of each intervening course  $C2$  across a three-needle spacing from the needle  $15A$  on which was formed a needle loop  $10n,14n$  in the formation of the preceding course  $C1$  to cause the yarns  $10,14$  to extend in a non-knitting manner about the spaced needle  $15B$ . Such needles  $15B$  hold the loop-forming yarns  $10,14$  during the formation of the intervening courses  $C2$  and then subsequently shed the yarns  $10,14$  without formation of needle loops thereof upon formation of the next succeeding alternate course  $C1$  and, since such needles are not involved in the formation of needle loops of the ground yarns  $12$  during the formation of any of the courses  $C1,C2$ , the held extents of the loop-forming yarns  $10,14$  do not become anchored in the fabric. As a result, the underlap extents  $14u$  of the second loop-forming yarns  $14$  are substantially elongated and are free to extend outwardly as pile-like loops from the corresponding face of the fabric, i.e. the technical back thereof. Likewise, the underlap extents  $10u$  of the first loop-forming yarns  $10$  are elongated and free to extend outwardly from the corresponding face of the fabric, i.e., the technical face, as more fully explained below.

In this fashion, the ground yarns  $12$  form a base or ground fabric structure which integrates the yarns  $10,12,14$  into the fabric, the coursewise alternating stitch construction of the ground yarns  $12$  permitting a corresponding degree of walewise stretchability of the fabric.

The formation of the loop-forming yarns  $14$  on the top (front) guide bar of the knitting machine forms such yarns predominantly at the technical back of the fabric whereat the extended underlaps  $14u$  extend generally outwardly of the fabric surface in the nature of elongated terry pile loops. Because of the particular stitch construction of the loop-forming yarns  $14$ , the successive underlap loops  $14u$  of each yarn  $14$  are formed during opposing lateral movements of the top guide bar and therefore the underlap loops  $14u$  in the resultant fabric tend to lean coursewise alternately in opposite directions relative to the needle loops  $14n$ , as depicted in FIGS. 1 and 2. As a result, the underlap loops  $14u$  produced by the present fabric construction make the fabric well suited for use as the loop component of a hook-and-loop fastener, the outwardly extending disposition of the underlap loops  $14u$  orienting them optimally for engagement with the hook elements of a mating fastener hook component, which could be of a variety of conventional constructions. Advantageously, the elongated nature of the underlap loops  $14u$  provides sufficient loop elevation from the fabric surface that napping, brushing or other mechanical raising of the loops, which is conventionally necessary in other fastener loop fabric constructions, can be avoided altogether.

The formation of the loop-forming yarns  $10$  on the bottom (back) guide bar of the knitting machine forms

such yarns predominantly at the technical face of the fabric. Thus, although the underlaps  $10u$  would normally tend to appear at the technical back of the fabric, because of the presence of the ground structure formed by the ground yarns  $12$ , the underlaps  $10u$  are caused to project from the technical face of the fabric, but to a lesser projecting elevation than the loops  $14u$  of the first loop-forming yarns  $14$  at the technical back. Since the underlaps  $10u$  of the second loop-forming yarns  $10$  are always formed during lateral movements of the bottom guide in the same direction, then in contrast to the loops  $14u$  of the yarns  $14$ , the underlap loops  $10u$  in the resultant fabric tend to project in the same direction as each other, thereby forming a walewise ribbed effect at the technical face of the fabric. Advantageously, the projecting loops  $10u$  facilitate adhesion of the technical face of the fabric to a substrate or backing material, leaving the technical back exposed to serve a fastening function, as more fully explained below.

FIG. 3 illustrates an alternative embodiment of the present textile fabric which is warp knitted of a two-bar construction on a two-bar weft insertion warp knitting machine according to the present method. In this embodiment, as in the embodiment of FIGS. 1 and 2, the top guide bar of the machine is threaded on alternating guide members in a "one out, one in" threading arrangement with a set of loop-forming yarns  $114$ , while the bottom guide bar is threaded on alternating guide members in a "one in, one out" threading arrangement with a set of ground yarns  $112$ . The top guide bar manipulates the set of loop-forming yarns  $114$  as they are fed from their respective warp beam to traverse relative to the needle bar alternately to stitch the loop-forming yarns  $114$  on alternating needles  $15A$  and then to lay the yarns  $114$  without stitch formation about spaced intervening needles  $15B$  in a repeating 1-0, 3-4, 6-7, 3-4 stitch pattern as indicated at II of FIG. 3. Simultaneously, the bottom guide bar of the knitting machine manipulates the set of ground yarns  $112$  as they are fed from their respective warp beam to traverse relative to the needle bar to stitch the ground yarns  $112$  on the same alternating needles  $15A$  in a repeating 1-0, 2-3, stitch pattern, as indicated at I in FIG. 3. The warp knitting machine includes a weft insertion device supplied with the filling yarn  $116$ . As the guide and needle bars of the knitting machine are manipulated to form each successive fabric course of the fabric, the weft insertion device is activated during the formation of each alternating course  $C1$  to insert the filling yarn  $116$  weftwise through the needle loops  $112n,114n$  of the ground and loop-forming yarns  $112,114$  and during the formation of the intervening courses  $C2$  to insert the filling yarn  $116$  weftwise through the needle loops  $112n$  of the ground yarn  $112$ .

Thus, the ground and loop-forming yarns  $112,114$  are inter-knitted with one another by formation of respective needle loops  $112n,114n$  of the yarns in alternating wales  $W1$  and alternating courses  $C1$  of the resultant fabric, without any needle loops of either of the yarns being formed in the intervening wales  $W2$  and only needle loops  $112n$  of the ground yarns  $112$  being formed in the alternating wales  $W1$  of the intervening courses  $C2$ . Specifically, the ground yarns  $112$  are formed only in the alternating wales  $W1$ , each individual ground yarn  $112$  having its respective needle loops  $112n$  alternating every course  $C$  between adjacent alternate wales  $W1$  across the one intervening wale  $W2$  across which underlaps  $112u$  of the ground yarn extend diagonally back and forth in a substantially coursewise direction

between the successive needle loops 112n. The stitch construction of the loop-forming yarns 114 form them in needle loops 114n appearing only in the alternating courses C1 and in the alternating wales W1, each individual loop-forming yarn 114 having its respective needle loops 114n formed in the alternating courses C1 in a single common wale W1 with connecting underlap extents 114u extending between the successive needle loops 114n generally in the intervening courses C2. The weftwise insertion of the filling yarns 116 cause them to extend coursewise back and forth across the fabric in parallel extents through the needle loops 112n, 114n in each succeeding fabric course C1, C2. As in the embodiment of FIGS. 1 and 2, the loop-forming yarns 114 appear predominantly at the technical back of the fabric whereat the elongated underlaps 114u are free to extend generally outwardly of the fabric surface in the nature of elongated terry pile loops, with the successive underlap loops 114u of each loop-forming yarn 114 tending to lean coursewise alternately in opposite directions relative to the needle loops 114n, making the fabric of FIG. 3 equally well suited for use as the loop component of a hook-and-loop fastener.

In use, the fabrics of the present invention provide several distinct advantages over conventional fastener loop fabric construction. By selecting the ground and loop-forming yarns to be of relatively fine denier, the present fastener loop fabric constructions can be made significantly lighter in weight per unit fabric dimension than corresponding conventional fastener loop fabric constructions. Further, manufacture of the present fabric constructions is expedited and simplified by avoiding the necessity of brushing, napping or otherwise raising the fastener loops 14u, 114u. As a result, the manufacturing cost of the present fabrics can be relatively reduced in comparison to conventional fastener loop fabrics. While the number of available fastener loops 14u, 114u provided by the present fabric constructions may be relative reduced in comparison to conventional fastener fabric constructions, the elongated upstanding nature of the loops 14u, 114u formed by the present constructions together with the opposing coursewise leaning of the loops provides optimal interengagement between the loops and the hook elements of a mating hook-type fastener component so that the peel force value, i.e., the force required to peel a hook fabric component from the present loop fabric, and the shear force value, i.e., the force required to pull a hook fabric component from the present loop fabric component in a direction parallel to the loop fabric component, compare favorably with conventional fastener loop fabric constructions.

Accordingly, the fastener loop fabric constructions of the present invention, owing to their provision of suitable functional characteristics at relatively lower cost and lighter weight than conventional fastener loop fabric constructions, are believed to be highly suitable for various forms of one-time and disposable uses such as, for example, use as a carpet backing of the type contemplated in aforementioned U.S. Pat. No. 4,822,658.

In particular, when the embodiment of the present fabric of FIGS. 1 and 2 is used as a carpet backing as disclosed in U.S. Pat. No. 4,822,658, the ribbed formation of the projecting loops 10u at the technical face of the fabric enable the fabric to be adhesively anchored by such loops in the foamed backing material of conventional carpets without necessarily adhering the ground structure of the present fabric in the carpet backing, whereby the natural walewise stretchability of

the present fabric is not inhibited thus permitting the fabric to stretch and move relative to the carpet and its backing so that the adherence of the present fabric to the carpet does not affect the normal performance characteristics of the carpet.

Alternatively, as depicted in FIG. 3, it is contemplated that the present fabric may be of a two-bar construction with pile-like loops appearing at only one face of the fabric, e.g., the loops 114u at the technical back of the fabric. In this case, however, since the opposite face of the fabric, i.e., the technical face, will necessarily need to be bonded directly to the foamed backing material of a carpet in the absence of anchoring loops such as the loops 10u in the fabric of FIGS. 1 and 2, it is believed to be important to minimize the degree to which the foam penetrates the interstices of the fabric's ground structure when bonding the fabric and foam together so that the natural walewise stretchability of the fabric will be substantially retained. Also, because the fastener fabrics of the present invention are inherently lighter in weight and more stretchable than conventional fastener fabrics, it has been found that the present fabrics are somewhat more difficult to handle during fabric finishing processes. Accordingly, the present invention also provides a method of treating the present fastener fabric preparatory to the performance of conventional fabric finishing processes to improve the fabric's handleability and to enable the fabric to sufficiently restrict foam penetration.

Specifically, the process of the present invention provides for application of a stiffening agent to the fabric to temporarily improve the handleability of the fabric, but it is contemplated that the stiffening agent should be readily broken and releasable from the fabric as a result of manipulation, bending and like handling of the fabric so that the stiffening agent does not remain as a permanent additive to the fabric and, in turn, the lengthwise stretchability of the fabric is not permanently impaired. A starch material performs suitably for this purpose, preferably a polyvinyl acetate (PVA) starch such as the Resin 5904 manufactured and sold by Cybron, Inc. of Wellman, S.C., formerly National Starch Corp. The starch is prepared in the form of a bath wherein the starch content is between approximately 10 percent and 40 percent of the total weight of the bath, the particular percentage being varied in relation to the method by which the starch is applied to the fabric and the resultant degree of starch take-up by the fabric accomplished by the application method. For example, the starch bath may be sprayed onto the technical face of the fabric, which advantageously minimizes the application of the starch to the fastener loops at the technical back of the fabric. In this case, a higher starch content in the bath near the upper end of the aforesaid range is preferable. Alternatively, the fabric may be passed through the bath in a conventional padding operation wherein the entire fabric is submerged in the bath, in which case a lower starch content near the lower end of the aforementioned range can be utilized.

In the present process, a foam resistant agent is also applied to the fabric to enable it to partially resist adhesion of the foam to the fabric and thereby to restrict foam penetration into the fabric structure so that the fabric retains a desirable degree of its lengthwise stretchability after adhesion to the foam backing layer of a carpet. Conventionally, urethane foam is predominantly used to produce the foam backing on conventional carpeting materials and, accordingly, the present

invention contemplates that a preferable foam resistant agent is a fluorocarbon surface finish. Furthermore, since urethane foam conventionally has both water and oil as constituent ingredients, the fluorocarbon composition should exhibit both water resistant and oil resistant properties, preferably accomplished by mixing a water-resistant fluorocarbon with an oil resistant fluorocarbon to produce the present fluorocarbon composition. The fluorocarbon composition is also produced in the form of a bath and, as will be understood, the fluorocarbon content of the bath should be carefully regulated so that the amount of fluorocarbon applied to the fabric will not be so great as to prevent any adherence of the fabric to the foam but at the same time it is not so small that the foam will still readily penetrate the interstices of the fabric's knit structure. Another factor that will affect the particular fluorocarbon content which is optimal in a given processing environment is the manner in which the foam is applied (e.g., the foam may be cast directly onto the technical face of the traveling fastener fabric and the carpet later adhered to the foam or, alternatively, the foam could be applied to the back of the traveling carpet and then the technical face of the fastener fabric laid onto the foam layer) and also the distance the fastener fabric must travel from the point at which the foam is applied to the point at which the foam cures. Generally, the fluorocarbon composition should have a total fluorocarbon content varying between approximately 0.25 percent and 8 percent of the total weight of the bath.

It will be recognized by those persons skilled in the art that the particular yarns and yarn sizes (denier), as well as the particular stitch patterns followed by the constituent yarns, may be selectively varied, as desired, to modify the properties and characteristics of the resultant fabric to achieve differing embodiments of the fabric suited to differing uses, so long as the stitch construction of the several yarns in selected to achieve elongated underlaps of the loop-forming yarns which are not anchored into the fabric structure so as to permit the underlaps to extend outwardly from the resultant fabric in the nature of pile loops. Likewise, it is contemplated that the fastener loop fabric of the present invention could be of a four bar construction rather than a three bar construction, if desirable to achieve additional or different fabric properties. All such modifications and variations on the present invention are intended to be within the scope of the present invention.

It will therefore be readily understood by those persons skilled in the art that the present invention is susceptible of a broad utility and application. Many embodiments and adaptations of the present invention other than those herein described, as well as many variations, modifications and equivalent arrangements will be apparent from or reasonably suggested by the present invention and the foregoing description thereof, without departing from the substance or scope of the present invention. Accordingly, while the present invention has been described herein in detail in relation to its preferred embodiment, it is to be understood that this disclosure is only illustrative and exemplary of the present invention and is made merely for purposes of pro-

viding a full and enabling disclosure of the invention. The foregoing disclosure is not intended or to be construed to limit the present invention or otherwise to exclude any such other embodiments, adaptations, variations, modifications and equivalent arrangements, the present invention being limited only by the claims appended hereto and the equivalents thereof.

What is claimed is:

1. A warp knitted textile fabric having one face of the fabric for adhering to a backing material and a set of loops extending from the opposite face of the fabric for mated engagement with hooking elements of another fabric for use in a two-component fabric fastener of a hook-and-loop type, said fabric comprising yarns formed in needle loops arranged in longitudinally extending wales and transversely extending courses including at least one set of ground yarns formed in a stitch pattern of needle loops which is stretchable in the walewise extent of the fabric and a set of loop-forming yarns knitted with said ground yarns in needle loops in spaced courses and spaced wales and in pile-like loops extending outwardly from said opposite face of said fabric.
2. A warp knitted textile fabric according to claim 1, wherein each said loop-forming yarn is formed in needle loops aligned with one another in spaced courses of a common wale.
3. A warp knitted textile fabric according to claim 1, wherein each walewise adjacent pair of said needle loops of said loop-forming yarns are spaced by at least one intervening course and each coursewise adjacent pair of said needle loops of said loop-forming yarns are spaced by at least one intervening wale.
4. A warp knitted textile fabric according to claim 1, wherein said pile-like loops of said loop-forming yarns are elongated underlap loops which extend outwardly from the technical back of said fabric.
5. A warp knitted textile fabric according to claim 4, wherein said elongated underlap loops extend in opposite directions coursewise of said fabric.
6. A warp knitted textile fabric according to claim 1, wherein said pile-like loops extend outwardly from technical face of the fabric.
7. A warp knitted textile fabric according to claim 1, wherein said loop-forming yarns are warp knitted in a 1-0, 3-4, 6-7, 3-4 stitch pattern.
8. A warp knitted textile fabric according to claim 1, wherein said loop-forming yarns are warp knitted in a 1-0, 3-4 stitch pattern.
9. A warp knitted textile fabric according to claim 1, wherein said ground yarns are warp knitted in a 2-3, 1-0 stitch pattern.
10. A warp knitted textile fabric according to claim 1 and wherein said ground yarns are knitted in a 1-0, 2-3 stitch pattern.
11. A warp knitted textile fabric according to claim 1 and further comprising a weft inserted filling yarn in at least some of said courses.
12. A warp knitted textile fabric according to claim 11 and wherein said weft inserted filling yarn extends coursewise in substantially every course.

\* \* \* \* \*